

## UNITED STATES PATENT OFFICE

2,271,324

## FLUSHING PIGMENTS

Edward G. Yee, Chicago, Ill., assignor to The Sherwin-Williams Company, Cleveland, Ohio, a corporation of Ohio

No Drawing. Application October 5, 1939,  
Serial No. 298,056

10 Claims. (Cl. 106—262)

The present invention relates to improvements in the manufacture of non-aqueous pigment dispersions in a liquefiable vehicle, and particularly to the transfer of aqueous pigment pulps directly into organic vehicles by an operation or process known to those skilled in the art as "flushing." It has special reference to agents for effecting and/or facilitating the transfer.

It is well known that some pigments may be flushed into oil without an added flushing agent. For example, aqueous white lead is readily flushed into linseed oil by simply mixing the two materials. Pigments in this class are usually hydrophobic in character. It is also known that certain agents facilitate the flushing operation, or even bring it about in the case of certain combinations of pigments and receiving vehicle. Pigments which do not flush easily or require agents to effect the transfer, are hydrophilic in character. Various explanations are given for the success of such agents or class of agents and for the failure of chemically similar compounds. Some of these explanations involve the physical nature of the molecule as well as its chemical reactivity.

The present invention is based upon the discovery that a group of amines not heretofore known as flushing agents are useful as such. The value of the invention lies in the facts that a relatively small quantity is needed to effect the transfer, and that the flushing agent is relatively inexpensive.

The object of the invention is to use as flushing agents amines or their soaps having the essential grouping



where R<sub>1</sub> and R<sub>2</sub> may be hydrogen, methyl, or benzyl groups, or combinations thereof.

It is also an object of the invention to form pigment dispersions characterized by the presence of a benzylamine flushing agent.

Other and ancillary objects and advantages will appear from the following description and explanation of the invention.

The invention may be used with both inorganic and organic pigments. The act of flushing involves intimate mixing of the aqueous pigment pulp and the receiving vehicle at a considerable expenditure of time and power. A flushing agent quickens the process and saves time and money. There is a frequent tendency of the vehicle and

water to emulsify in such operations. Hastening the process minimizes emulsification. The formation of emulsion decreases the efficiency of the flushing operation, because more water is retained in the mass, which water must be removed by other means. One use of the flushing agent is to minimize or prevent the formation of emulsion.

Pigments particularly suitable for flushing in accordance with this invention are iron blues, chrome yellows, organic lakes and pigment dyes-stuffs.

The vehicle may be any water-immiscible liquid or solid which is or becomes liquid at the temperature of operation. It may be selected from coal tar solvents, mineral spirits, hydrogenated naphthas, representing the volatile vehicles, or from linseed oil, China wood oil, soya bean oil, perilla oil, other vegetable and animal oils, synthetic and oleoresinous varnishes, representing the drying vehicles, or mineral oil, petrolatum, castor oil and waxes, representing the non-drying vehicles. All these may be used in the present invention. The drying oils ordinarily have an acid number, representing a content of fatty acid which may form a soap with the amine flushing agent. The formation of the soap does not render the amine ineffective, for the amine agent may be added effectively as a soap or as the free amine. The amine may be condensed with soap-forming fatty acids such as oleic, stearic, palmitic, linolenic, ricinoleic acid, or with soap-forming resin acids, such as rosin or abietic acid, to form the amine soap flushing agent.

Because the free amine or its soaps may be used with vehicles which are volatile or which possess no acid number, it is known that both the free amine and its soaps are flushing agents. While soap formation is not essential for the practice of this invention, some acidity in neutral vehicles adds to the effectiveness of the amine flushing agents, where the acid is of a soap-forming character. Thus, fatty acids or other soap-forming acids may be added.

Examples are given below to illustrate this invention. While these examples deal mainly with iron blue pigments, its usefulness is not restricted to such. Iron blue (ferric ferrocyanide) is highly hydrophilic and is one of the most difficult pigments to employ in a flushing process. Therefore, the invention is illustrated largely by reference to it, as it is the severest test found to measure the comparative effectiveness of the flushing agents.

EXAMPLE I  
Printing ink base

1667 lbs. of water-wet iron blue presscake containing 500 lbs. of the pigment (dry basis), 500 lbs. litho varnish (a heat-bodied linseed oil varnish), 15 lbs. benzylamine.

About one-third of the iron blue presscake and 250 lbs. of litho varnish are mixed in a machine of the dough-mixer type, equipped for vacuum drying, heating and cooling. Any machine that gives intimate mixing will serve as well. To this mixture is then added 9 lbs. of benzylamine and mixing continued. In a short time, usually less than twenty minutes, the water in the presscake will separate or "flush out" and the iron blue is taken up by the varnish. The water is decanted off or removed by other means, and about one third of the remaining presscake is added to the mixer. At this stage, 50 lbs. of litho varnish and 2 lbs. of benzylamine are also added. On further mixing, more water is flushed out. The remaining presscake is flushed out in two charges in the above manner, using 2 lbs. of benzylamine and 50 lbs. of litho varnish in each charge. When all the presscake is flushed, steam is turned on and the temperature of the mass raised to 50°-60° C. Vacuum is applied to the mixer and mixing is continued under reduced pressure until the pigment-oil paste is substantially water-free. The mass is cooled and the remaining 100 lbs. of litho varnish added to make a base ink containing one part of pigment to one part of varnish. This is a typical procedure for the practice of this invention, but it is not restricted to such. Those skilled in the art will vary this procedure to suit their own need. Instead of vacuum drying, the paste may be finished upon a roller mill. The time-cycle for this procedure is about four hours.

## EXAMPLE II

2000 lbs. of water-wet iron blue presscake containing 500 lbs. of the pigment (dry basis), 500 lbs. litho varnish, 25 lbs. dibenzylamine.

The procedure is similar to that of Example I.

## EXAMPLE III

2000 lbs. of water-wet iron blue presscake containing 500 lbs. of the pigment (dry basis), 500 lbs. mineral oil, 15 lbs. benzyl N-dimethyl amine, 25 lbs. oleic acid. The oleic acid and the benzyl dimethyl amine are mixed to form a benzylidemethyl olate soap with an excess of the free amine. From this point on, the procedure is similar to that of Example I. The amine soap and mineral oil are added to the mixer as needed.

## EXAMPLE IV

3000 lbs. of water-wet medium chrome yellow containing 2000 lbs. of the pigment (dry basis), 500 lbs. linseed oil, 10 lbs. benzylamine.

The procedure is similar to that of Example I.

## EXAMPLE V

2000 lbs. of water-wet iron blue presscake containing 600 lbs. of the pigment (dry basis), 800 lbs. of glycerol-phthalate varnish, 100% solids, 600 lbs. mineral spirits, 25 lbs. benzylamine.

The pigment is flushed in the glycerol-phthalate varnish with benzylamine, similar to Example I. The mass is vacuum dried and cooled, and the mineral spirits added.

The foregoing examples establish that the amine may be primary, secondary or tertiary, so

long as it has at least one benzyl radical. This establishes that the effective grouping is



in a free amine or in an amine soap. The agents may have solubility in water, but are generally more soluble in the liquid vehicle. The removal of water from the mass after a flushing operation may remove some of the agent. However, where the operation is conducted in one step, its main function has been performed. Where the operation is carried out in several steps more of the agent is added, so that any removal of some of the agent in the withdrawn water cannot be effective to deplete the process of the agent.

The oil pastes prepared in the manner described are suitable for the manufacture of all types of protective and decorative finishes, and for allied applications.

The quantity of flushing agent required for a given result varies with the apparatus used, the pigment, the pulp concentration, the receiving vehicle, and other factors. It is a small quantity, commonly less than 5% of the dry weight of pigment.

The practice may be varied in accordance with the scope of the invention as expressed in the appended claims.

I claim:

1. The method of flushing pigment particles from aqueous paste form into a liquid vehicle immiscible with water to release water, which comprises agitating a mass of aqueous pigment paste with a receiving liquid vehicle which is immiscible with water, in the presence of a small quantity of a benzylamine compound having the grouping therein with the formula



in which  $R_1$  and  $R_2$  may be selected from the group consisting of hydrogen, and the radicals: methyl and benzyl.

2. The method of flushing pigment particles from aqueous paste form into a liquid vehicle immiscible with water to release water, which comprises agitating a mass of aqueous pigment paste with a receiving liquid vehicle which is immiscible with water, in the presence of a small quantity of a benzylamine compound of the formula



in which  $R_1$  and  $R_2$  may be selected from the group consisting of hydrogen, and the radicals: methyl and benzyl.

3. The method of flushing pigment particles from aqueous paste form into a liquid vehicle immiscible with water to release water, which comprises agitating a mass of aqueous pigment paste with a receiving liquid vehicle which is immiscible with water, in the presence of a small quantity of a benzylamine soap of a benzylamine of the formula



in which  $R_1$  and  $R_2$  may be selected from the group consisting of hydrogen, and the radicals:

methyl and benzyl, and a soap-forming acid selected from the group of soap-forming resin acids and soap-forming fatty acids.

4. The method according to claim 1 in which the receiving liquid contains a drying vehicle for pigment.

5. The method according to claim 1 in which the receiving liquid is a non-drying vehicle for pigment.

6. The method according to claim 1 in which the receiving vehicle is volatile.

7. The method according to claim 1 in which one of the attachments  $R_1$  and  $R_2$  is hydrogen.

8. The method according to claim 1 in which the compound is benzylamine.

9. The method according to claim 1 in which the receiving liquid is litho varnish.

10. The method according to claim 1 in which the pigment is iron blue.

EDWARD G. YEE.